# EUROPEAN PATENT SPECIFICATION

(11) **EP 0 663 789 B1**
(45) Date of publication and mention of the grant of the patent: **15.12.1999**
(21) Application number: 94305456.9
(22) Date of filing: 22.07.1994
(51) Int. Cl.: H05B 41/29

(54) **Preheat start-up device for fluorescent lamps**
Vorheizstartschaltung für Leuchtstofflampen
Circuit d'amorçage, avec préchauffage, de lampes fluorescentes

(30) Priority: 18.01.1994 CN 94202144
(43) Date of publication of application: 19.07.1995
(73) Proprietor: MASS TECHNOLOGY (H.K.) LTD., Tsim Shatsui, Kowloon (HK)
(72) Inventor: Foo, Onn Fah, Tsim Sha Tsui, Kowloon (HK)
(74) Representative: Archer, Philip Bruce

(56) References cited:
- WO-A-93/00784

## Description

This invention relates to a discharge lamp preheating start-up device comprising a voltage-sensitive switching element and a temperature sensitive resistance having a positive temperature coefficient, and a method of producing such a device.

More particularly, the invention relates to a pre-heating start-up device for electronic ballast fluorescent lamps, and a method of producing same.

Fluorescent lamps have been widely used as an efficient lighting device and require, during normal operation, accessories such as current limiting means and start-up means. Current limiting means (ballast) frequently used are electronic and lamps using such current limiting means are known as high frequency lamps. These have the advantage of a low voltage start-up. The start-up means used as the operating switch in such lamps are the so-called "jumping bulb" glow starter. This is a monodirectional glow heat sensitive switch having a pair of head closing metallic electrodes sealed into a glass shell filled with an inert gas. The normal operative gas discharging voltage of the filament at the two ends of the fluorescent tube can be reached to cause glow of the light tube. This method of starting glow is known as high voltage quick cold start-up under normal temperature and does not involve any apparent pre-heating process of the filaments of the light tube during the starting procedure. Accordingly the light tube can only be started under high voltage conditions together with an impulse of high current (approximately 2.5 times the operating current of the lamp). Such high voltage quick cold starting may cause direct damage of the filament and the electron powder and may also cause the "rectifying effect" of asymmetric electron emitting, both affecting the life of the light tube.

More recently, fluorescent lamps have been developed which are gas charging lamps of the cathode preheating type, which are hot starting lamps. In order to prolong the life of a light tube it is important to "hot start" the light tube in preheating conditions, that is, the tube is lit at a relatively low open line voltage (such as at 300 to 400 volts instantaneous peak starting voltage) after a period of preheating the filaments. This is advantageous to prevent the filament and its superficial electron emitting material from "spurting out", whereby, the life of the light tube can be prolonged.

Heat sensitive resistors are relatively commonly adopted in making preheating type glow starters. This is a device having a positive temperature coefficient (PTC), which has been described in detail in US patent number 3,444,399. PTC thermistors have temperature sensitive characteristics and are directly used in electronic circuits to compensate for voltage change and to provide a stable current passing through the circuit load. Chinese Utility Model Patent number 92219487 discloses utilising a PTC in fluorescent lamp glow preheating. The fluorescent lamp starting preheater disclosed therein is a thermistor having a positive temperature coefficient and Curie point or switching temperature. The two terminals of the preheater are coupled to the two thermals of the main oscillatory circuit of the electronic ballast serially connected to the two filaments of the fluorescent lamp, respectively, as shown in Fig 1 hereof. It is necessary to match the parameters and volume of the PTC with the electronic parameters of the light tube when the PTC is utilised as a preheating device and this is difficult to achieve. In addition, the PTC itself also consumes power, its temperature rise is high and its starting time is relatively long (about three seconds).

A discharge lamp preheating start-up device comprising a voltage-sensitive resistance having a positive temperature coefficient is described in WO-A-93 00784. The resistance is interconnected in series with the bidirectionally operating breakdown voltage-sensitive switching element. The resistance and the bidirectionally operational breakdown element are thermally coupled. The purpose is to provide simple circuit for operating a discharge lamp which facilitates the substantially constant ignition of the lamp.

It is an object of the present invention to provide a fluorescent lamp preheating starter having both the characteristics of positive temperature resistance and the function of a voltage switch and/or to provide a fluorescent lamp preheating starter having suitable start-up time and easy matching with the electric parameters of the light tube; and/or to provide a fluorescent lamp preheating starter having low power consumption per se and low temperature rise; and/or to provide improvements generally.

According to the invention there is provided a preheating starter-up device for electronic ballast fluorescent lamps and a method of producing same as claimed in the accompanying claims.

In an embodiment of the invention there is provided a preheating start-up device for electronic ballast fluorescent lamps constructed in the following manner. Two materials are used. One (referred-to below as the "V" layer) of which comprises more than 80% zinc oxide with minor additions of oxides of bismuth, antimony, cobalt and manganese. The other one (referred-to below as the "T" layer) of which comprises a mixture of oxides comprising more than 70% by weight of a barium and strontium and titanium complex oxide. These materials are mixed, respectively, and compressed to form circular sheets of 4-7mm diameter, and shaped by sintering. Each of the two surfaces of each sheet is then coated with a conductive layer of silver, thereafter, the two sheets obtained are hot bonded into an integrated body to form a chip. In the chip, the portion comprising a complex oxide of (inter-alia) barium is designated the "T" layer, while the portion mainly comprising zinc oxide is designated the "V" layer. Connecting leads are led out from the surfaces of the two layers, respectively, and together they form a fluorescent lamp automatic preheating/switch device, referred to as a VT device. The VT device is serially connected into the fluorescent lighting circuit. The above-mentioned chip of the VT device is then sealed into a coating of burn - resistant epoxy powder with is integrated by heating to form a complete device. The fluorescent lamp automatic preheating/switching device thus formed is serially connected in the loop of the filament of the fluorescent lamp after the parallel connection of the two leads with a resonant capacitor.

The "V" layer in the VT device behaves as a voltage sensitive switching resistor, it operates as a voltage sensitive switch and increases the initial current, speeds up the variation of resistance of the "T" layer and improves the starting speed of the light tube. The "T" layer in the VT device behaves as a PTC, which functions to delay the rise of the voltage in the light tubes circuit and prevents the exceeded current from passing through the "V" layer.

The selection of materials constituting the VT device and the ranges of its electric parameters can be varied accordingly depending on the features of the lamps with which they are used.

In use, voltage is applied to the two terminals of a fluorescent lamp. As the cold state conducting voltage of the light tube is higher than 600V, when the conducting voltage of said VT device is only approximately 150V, the VT device is first made conductive at a relatively low voltage, thus, the two terminals of the VT device lower the peak voltage.

Since the voltage at the two terminals of the light tube is maintained only at the voltage value of the voltage sensitive switch of the VT device, that is approximately 180V, therefore the lamp is not conductive. During this period, the current in the whole circuit passing through the VT device (approximately 80 mA) and the charging and discharging currents of the resonant capacitor C heat the filaments, and at the same time, the VT device is also heated.

The resistance of the temperature sensitive device in the VT device increases with the rise of temperature, that is, the voltage of the two terminals of the light tube increases continuously ( V=IR), finally, when this voltage reaches the heat conducting voltage of the tube, ie 300 to 400V, the light tube becomes conductive and the gas inside the tube discharges, subsequently the voltage at the two terminals of the light tube or the two terminals of the VT device lowers to the normal working voltage of the light tube, ie approximately 70-90V, and at this stage the VT device converts to an "off" state.

Thus, in spite of the fact that there is a capacitance of about 350 PF in the VT device together with an internal resistance of about 1kW, there will still be a weak current under the high frequency power supply. During the passing through of these currents in the VT device, there will be a power consumption of about 0.015 Watt, but as compared with the self-power-consumption of ordinary PTC (approximately 0.4 Watt), it has been greatly reduced.

When the fluorescent lamp preheating starter of the embodiments is utilised, in addition to the fact that the temperature controlled impedance feature of ordinary PCT is maintained, there is also the function of a voltage switch, thereby, the power consumption of the preheating starter of the present invention during the normal working period of the fluorescent lamp is only 0.4 to 5% of that of the PTC.

The consequent advantages are that the rise of temperature of said device is low, it is easy to realise parameter matching with the light tube and the starting time is also appropriate. The reliability of the operation of the light tube can be improved, and the life of the light tube can be prolonged.

Embodiments of the invention will now be described by way of example only with reference to the accompanying illustrative drawings in which :
Fig 1 shows a circuit diagram showing a fluorescent lamp utilizing the prior art PTC preheating starting device;
Fig 2 shows a circuit diagram showing a fluorescent lamp utilising the VT preheating starting device of the present invention;
Fig 3 is a schematic drawing showing the structure of the VT preheating starting device of the present invention; and
Fig 4 is a schematic drawing showing a modification of the VT preheating starting device of the present invention.

As shown in Fig 2, the device indicated by the symbol VT is a fluorescent lamp preheating starting device or automatic glow starter/switch device of the present invention, which constitutes a serial circuit with the electronic ballast and the filaments and is connected in parallel with the resonant capacitor C.

Fig 3 shows a schematic diagram illustrating the structure of a fluorescent lamp preheating starting device, wherein the temperature sensitive resistance layer or "T" layer or sheet 1 comprises a mixture of oxides comprising more than 70% by weight of a barium and strontium and titanium complex oxide. In this embodiment the complex oxide has the molecular formula (0.878 Ba + 0.122 Sr + Ti) 0₃. The mixture contains oxides in the proportions given by one mole of this latter oxide mixed with the mole percentages now indicated of the following additional oxides : 0.05-0.3mol% NB₂O₅ and 0.8-3mol% SiO2 and 0.2-0.8mol% Al203 and 0.4-1.5mol% TiO2 and 0.03-0.08mol%CaO and 0.005 (or 0.05) - 0.01mol% MnO2 and 0.04-0.8mol%MgO.

The resistance layer has the properties of a heat sensitive resistor and is coated with a conductive layer, the Curie Point of which is 60°C to 100°C, and its resistance at normal temperature is 700 to 1200 . It corresponds to an MZ11PTC heat sensitive resistor.

The voltage sensitive switching resistance V layer or sheet 2 comprises a mixture comprising more than 80% zinc oxide with minor additions of oxides of bismuth, antimony, cobalt and manganese. In this embodiment the molecular percentages are as follows : 95-98mol% ZnO plus 0.1-5mol% of each of Bi2O, Sb2O3, CoO and MnO.

The V layer or sheet is a voltage sensitive structure, the voltage value of the voltage sensitivity is 120-160 volts, and the mean features of which are similar to that of an MYD-07K95 voltage sensitive resistor.

One surface of this voltage sensitive switching resistance layer (sheet) 2 is hot bonded with the above-mentioned temperature sensitive resistance layer (sheet) 1 by solder 4. Said solder is a tin plated brass wire solder attached with D4D-87 silver epoxy conductive glue. The thickness of the silver layer is 0.06 mm and being able to withstand temperatures of 300°C, it is in fact a conductive layer. Leads 3 are connected to the temperature sensitive resistance layer (sheet) 1 and the voltage sensitive switching resistance layer (sheet) 2 respectively. The two layers 1 and 2 are hot bonded together to form an integrated body.

The above apparatus is sealed by a coating film 5 comprising epoxy powder to form an automatic starter/switch VT device having both temperature controlled impedance characteristics and voltage switching characteristics.

The main parameters of the automatic starter/switch VT device are as follows :
Switching voltage : 120 to 160 Volt
Curie point : 65°C to 100°C
Internal resistance (normal temperature) : 700 Ω to 1200 Ω.
Temperature resistance coefficient : >(R-700)10%/1°C (positive characteristic)
Power consumption : <0.03 Watt (during normal operation of the light tube)
Starting time : 0.6 to 1.5 sec (under normal temperature)
Life of switch : 100,000 times (under normal temperature)
Withstand voltage : >1000 Volt
Static capacitance : <350 PF

The above-mentioned materials constitute a fluorescent lamp starting device having both the function of a voltage switch and the characteristic of self-overload-current-protection, which is capable of automatic preheating, automatic switching, and self-protection. The lamp starting time of this automatic preheating/switching device (VT) is appropriate, ie 0.6 to 1.5 second, the life of the switch can be controlled in 20,000 to 100,00 times.

Fig 4 illustrates an embodiment of another structure of the fluorescent lamp preheating starter of the present invention as a modification of the above-mentioned structure. Therein, a current limiting resistance film 6 in parallel with the temperature sensitive device is coated on the peripheral (one or more peripheral surfaces) thereof. On the basis of the basic structure of the above-mentioned VT device, the resistance of this film is 12K Ohms to 20K Ohms. A current limiting resistor having the same resistance range may also be connected in parallel with the temperature sensitive device.

A further embodiment of the VT device of the present invention is one in which the voltage sensitive resistance layer (sheet) 2 and the temperature sensitive resistance layer (sheet) 1 in the above-mentioned structure are made separated, and the same effect is achieved merely by connecting them in series with a conductor and then mounting them in the location indicated by VT as shown in Fig 2.

## Claims

1. A discharge lamp preheating start-up device comprising a voltage-sensitive switching element and a temperature-sensitive resistance having a positive temperature coefficient, characterised in that
hot bonded into an integrated body with the voltage-sensitive switching element comprising a switching resistance layer (2) comprising more than 80% zinc oxide together with the temperature-sensitive resistance comprising a layer (1) comprising a mixture of oxides comprising more than 70% by weight of a barium and strontium and titanium complex oxide, there is provided a silver-coated conductive layer between said two resistance layers (2,1), said device having leads (3) and said layers (2,1) being sealed into a coating film (5) to form an automatic preheating/switching device.

2. A start-up device according to claim 1 characterised in that the diameter of said two resistance layer (2,1) is approximately in the range of 4mm to 7 mm.

3. A start-up device according to claim 1 or claim 2 characterised in that said voltage-sensitive resistance layer (2) and said temperature-sensitive resistance layer (1) are separate devices connected in series by a conductor.

4. A start-up device according to any one of claims 1 to 3 characterised in that the periphery of said temperature-sensitive layer (1) is coated with a current-limiting resistance film (6) coupled in parallel therewith.

5. A start-up device according to any one of claims 1 to 3 characterised in that a current-limiting resistor is connected in parallel with said temperature-sensitive layer (1).

6. A start-up device according to any one of claims 1 to 5 characterised in that the voltage-sensitive resistance value of said voltage-sensitive switching device lies in the range of 120 volts to 160 volts.

7. A start-up device according to any preceding claim characterised in that said temperature-sensitive resistance layer comprises a mixture comprising titanium oxide, the Curie point thereof lying in the range from 65°C to 100°C, and the resistance under normal temperatures being from 700 Ohms to 1200 Ohms.

8. A start-up device according to any one of the preceding claims characterised in that said oxide comprising barium is a complex oxide of barium strontium and titanium.

9. A start-up device according to any one of the preceding claims characterised in that the oxide comprising barium is a barium carbonate.

10. A method of producing a discharge lamp preheating start-up device comprising a voltage-sensitive switching element and a temperature resistance having a positive temperature coefficient, characterised in that
the voltage-sensitive switching element is a layer (2) comprising more than 80% zinc oxide compressed to form a circular sheet of 4mm to 7mm diameter and shaped by sintering, that the temperature-sensitive resistance is a layer (1) comprising a mixture of oxides comprising more than 70% by weight of a barium and strontium and titanium complex oxide compressed to form a circular sheet of 4mm to 7 mm diameter and shaped by sintering, that leads (3) are connected to the temperature-sensitive resistance layer (1) and the voltage-sensitive switching resistance layer (2) respectively and that the two layers (1, 2) are hot bonded by a silver conductive layer to form an integrated body.

## Patentansprüche

1. Leuchtstofflampen-Vorheizstartvorrichtung, umfassend ein spannungsempfindliches Schaltelement und einen temperaturempfindlichen Widerstand mit einem positiven Temperaturkoeffizienten, dadurch gekennzeichnet, daß heißkontaktiert bzw. verbunden in einem integrierten Körper mit dem spannungsempfindlichen Schaltelement, welches eine Schalt-Widerstandsschicht (2), mit mehr als 80 % Zinkoxid, umfaßt, gemeinsam mit dem temperaturempfindlichen Widerstand, welcher eine Schicht (1) aus einer Mischung von Oxyden mit mehr als 70 Gew.% eines Barium- und Strontium- und Titan- Komplexoxydes bzw. Mischoxydes umfaßt, eine silberbeschichtete, leitfähige Schicht zwischen den zwei Widerstandsschichten (2, 1) vorgesehen ist, wobei die Vorrichtung Anschlüsse (3) aufweist und die Schichten (2, 1) in einem Beschichtungsfilm (5) versiegelt sind, um eine automatische Vorheiz/ Schalt-Vorrichtung zu bilden.

2. Startvorrichtung nach Anspruch 1, dadurch gekennzeichnet, daß der Durchmesser der zwei Widerstandsschichten (2, 1) ungefähr im Bereich von 4 mm bis 7 mm liegt.

3. Startvorrichtung nach Anspruch 1 oder 2, dadurch gekennzeichnet, daß die spannungsempfindliche Widerstandsschicht (2) und die temperaturempfindliche Widerstandsschicht (1) getrennte Vorrichtungen sind, welche in Serie miteinander durch einen Leiter verbunden sind.

4. Startvorrichtung nach einem der Ansprüche 1 bis 3, dadurch gekennzeichnet, daß der Umfang der temperaturempfindlichen Schicht (1) mit einem strombegrenzenden Widerstandsfilm (6), welcher parallel damit gekoppelt ist, beschichtet ist.

5. Startvorrichtung nach einem der Ansprüche 1 bis 3, dadurch gekennzeichnet, daß ein strombegrenzender Widerstand parallel mit der temperaturempfindlichen Schicht (1) verbunden ist.

6. Startvorrichtung nach einem der Ansprüche 1 bis 5, dadurch gekennzeichnet, daß der spannungsempfindliche Widerstandswert der spannungsempfindlichen Schaltvorrichtung in dem Bereich von 120 V bis 160 V liegt.

7. Startvorrichtung nach einem der vorangehenden Ansprüche, dadurch gekennzeichnet, daß die temperaturempfindliche Widerstandsschicht eine Mischung, umfassend Titanoxid, umfaßt, deren Curiepunkt im Bereich vom 65 °C bis 100 °C liegt, und daß der Widerstand bei normalen Temperaturen von 700 Ohm bis 1200 Ohm beträgt.

8. Startvorrichtung nach einem der vorangehenden Ansprüche, dadurch gekennzeichnet, daß das Barium-enthaltende Oxid ein komplexes Oxid von Barium, Strontium und Titan ist.

9. Startvorrichtung nach einem der vorangehenden Ansprüche, dadurch gekennzeichnet, daß das Barium-enthaltende Oxid ein Bariumcarbonat ist.

10. Verfahren zur Herstellung einer Leuchtstofflampen-Vorheizstartvorrichtung, umfassend ein spannungsempfindliches Schaltelement und einen Temperaturwiderstand mit einem positiven Temperaturkoeffizienten, dadurch gekennzeichnet, daß das spannungsempfindliche Schaltelement eine Schicht (2), mit mehr als 80 % Zinkoxid, ist, welche komprimiert wird, um ein kreisförmiges Blatt mit einem Durchmesser von 4 mm bis 7 mm auszubilden, und durch Sintern geformt wird, daß der temperaturempfindliche Widerstand eine Schicht (1), mit einer Mischung von Oxyden mit mehr als 70 Gew.% eines Barium- und Strontium- und Titan- Komplexoxydes bzw. Mischoxydes umfaßt, welche komprimiert wird, um ein kreisförmiges Blatt mit einem Durchmesser von 4 mm bis 7 mm auszubilden, und durch Sintern geformt wird, daß Anschlüsse (3) mit der temperaturempfindlichen Widerstandsschicht (1) bzw. der spannungsempfindlichen Schalt-Widerstandsschicht (2) verbunden werden und daß die zwei Schichten (1, 2) durch eine leitfähige Silberschicht heißkontaktiert bzw. verbunden werden, um einen integrierten Körper zu bilden.

## Revendications

1. Dispositif d'amorçage avec préchauffage pour lampe à décharge, comprenant un élément de commutation sensible à la tension et une résistance sensible à la température ayant un coefficient de température positif, caractérisé en ce que, liée à chaud en un corps intégré avec l'élément de commutation sensible à la tension, comprenant une couche de résistance de commutation (2) qui contient plus de 80% d'oxyde de zinc, et avec la résistance sensible à la température comprenant une couche (1) d'un mélange d'oxydes qui contient plus de 70% en poids d'oxyde complexe de baryum, strontium et titane, il est prévu une couche conductrice à revêtement d'argent entre lesdites deux couches de résistance (2, 1), ledit dispositif comportant des conducteurs (3) et les dites couches (2,1) étant scellées dans un film de revêtement (5) pour constituer un dispositif de préchauffage/ commutation automatique.

2. Dispositif d'amorçage selon la revendication 1, caractérisé en ce que le diamètre desdites deux couches de résistance (2,1) est approximativement dans la plage de 4 mm à 7 mm.

3. Dispositif d'amorçage selon la revendication 1 ou la revendication 2, caractérisé en ce que la dite couche de résistance sensible à la tension (2) et ladite couche de résistance sensible à la température (1) sont des dispositifs séparés connectés en série par un conducteur.

4. Dispositif d'amorçage selon une quelconque des revendications 1 à 3, caractérisé en ce que la périphérie de ladite couche sensible à la température (1) est revêtue avec un film de résistance de limitation de courant (6) couplé en parallèle avec elle.

5. Dispositif d'amorçage selon une quelconque des revendications 1 à 3, caractérisé en ce qu'une résistance de limitation de courant est connectée en parallèle avec ladite couche sensible à la température (1).

6. Dispositif d'amorçage selon une quelconque des revendications 1 à 5, caractérisé en ce que la valeur de résistance sensible à la tension dudit dispositif de commutation sensible à la tension est dans la plage de 120 volts à 160 volts;

7. Dispositif d'amorçage selon une quelconque des revendications précédentes, caractérisé en ce que la dite couche de résistance sensible à la température comprend un mélange contenant de l'oxyde de titane, dont le point de Curie est situé dans la plage de 65°C à 100°C, et la résistance dans des conditions de température normale est de 700 Ω à 1200 Ω.

8. Dispositif d'amorçage selon une quelconque des revendications précédentes, caractérisé en ce que le dit oxyde contenant du baryum est un oxyde complexe de baryum, strontium et titane.

9. Dispositif d'amorçage selon une quelconque des revendications précédentes, caractérisé en ce que l'oxyde contenant du baryum est un carbonate de baryum.

10. Procédé de fabrication d'un dispositif d'amorçage avec préchauffage pour lampe à décharge, comprenant un élément de commutation sensible à la tension et une résistance sensible à la température ayant un coefficient de température positif, caractérisé en ce que l'élément de commutation sensible à la tension est une couche (2) contenant plus de 80% d'oxyde de zinc comprimée pour former une feuille circulaire de 4 mm à 7 mm de diamètre etmise en forme par frittage, en ce que la résistance sensible à la température est une couche (1) comprenant un mélange d'oxydes qui contient plus de 70% en poids d'oxyde complexe de baryum, strontium et titane, comprimée pour former une feuille circulaire de 4 mm à 7 mm de diamètre et mise en forme par frittage, en ce que des conducteurs (3) sont connectés à la couche de résistance sensible à la température (1) et à la couche de résistance de commutation sensible à la tension (2) respectivement, et en ce que les deux couches (1,2) sont liées à chaud par une couche conductrice en argent pour former un corps intégré.
